

Nov. 5, 1940.

A. HENDERSON

2,220,448

METHOD OF MAKING CONCRETE BLOCKS AND THE LIKE

Filed Aug. 5, 1938



INVENTOR  
Albert Henderson  
by his attorney  
Stalbin, Blanks  
& Parmelee

## UNITED STATES PATENT OFFICE

2,220,448

METHOD OF MAKING CONCRETE BLOCKS  
AND THE LIKEAlbert Henderson, Edgewood, Pa., assignor to  
William P. Witherow, Pittsburgh, Pa.

Application August 5, 1938, Serial No. 223,300

5 Claims. (Cl. 25—155)

This invention relates to the manufacture of molded cementitious articles such as blocks, slabs, etc., and, particularly, to a method of making such articles whereby they may be produced 5 more cheaply than heretofore and at the same time be characterized by superior quality.

This is a continuation in part of my copending application, Serial No. 62,965, filed February 8, 1936, for Apparatus for making concrete articles, 10 now Patent No. 2,131,474, granted September 27, 1938.

Concrete blocks and the like have usually been made heretofore by the so-called dry process. While this process produces blocks which are 15 satisfactory for many uses such as foundation walls and the like where appearance is a secondary consideration, the blocks so made have not been used widely in exposed locations. Further objections to the previous method of making 20 blocks include the high labor cost resulting from the necessity for handling the blocks individually from the molds to storage piles, as well as the danger of chipping and breakage resulting from such handling. The prior practice has been to 25 store the blocks for aging in any convenient place, without protection from the weather or changes in atmospheric temperature. This causes discoloration of the blocks and renders them generally undesirable from the standpoint 30 of appearance.

I have invented a novel method of making blocks and similar articles of concrete which overcomes the aforementioned objections and is characterized by further features of advantage 35 and novelty which will become apparent as the following detailed description of the invention proceeds. In a preferred practice of the invention, I pour liquid concrete into gang molds, preferably from a traveling hopper. The hopper 40 may conveniently be supplied with concrete from a truck mixer. The blocks or other articles are partly cured in the mold and then removed therefrom to a curing chamber for final curing. After curing, the blocks are dipped to chill them 45 and stored in the same room where molded and cured whereby the waste heat from the molding and curing operations prevents the blocks from being subjected during aging to dangerously low temperatures. A complete understanding of the 50 invention may be obtained from the following description which is to be read with reference to the accompanying drawing in which the figure is a transverse sectional view through a block manufacturing plant arranged to operate in accordance with the invention.

Referring in detail to the drawing, I prefer to carry out the molding, curing and aging of blocks within a single room or building as indicated by side walls 10, roof 11 and suitable end walls. A bridge crane 12 traversing the length 5 of the building facilitates transfer of the blocks from point to point therein.

An aisle 13 extends the length of the building, conveniently along one side thereof, and is provided with a paved roadway 14 for the passage 10 therealong of a vehicle adapted to deliver mixed concrete, the usual form of such vehicle being a truck mixer as indicated diagrammatically at 15. As is well-known, these vehicles are charged with sand, cement, aggregate and water at central batching plants and effect the necessary mixing of such materials while en route to the point of delivery.

Molding apparatus indicated generally at 16 is arranged alongside the aisle 13. This apparatus is preferably such as that more fully described and claimed in the parent application above referred to. Briefly, it comprises side rails 17 along which a traveling hopper 18 moves. Gang molds 19 are spaced along the side rails 20 and adapted to receive concrete from the hopper in its various positions as it travels along the rails. A water tank 20 is installed beneath the gang molds and is provided with steam pipes 21 whereby heat and moisture may be supplied to 25 the space surrounding the molds.

In accordance with the invention, concrete is discharged from the truck mixer 15 to the hopper 18 through a chute 22 periodically or continuously as may be desired. The hopper 18 discharges concrete to one gang mold 19 until the latter is filled to the desired level. Thereupon the truck mixer and hopper are moved along the aisle to the next gang mold. If desired, a coupling may be provided between the mixer and 35 hopper so that the hopper is drawn along the side rails 17 by the truck mixer in the manner of a trailer.

After the mold 18 has been filled, it is subjected to vibration by any suitable means to 40 densify and compact the concrete in the several mold chambers. Steam is then admitted to the pipes 21 in such manner as to maintain the temperature adjacent the mold at about 175° F. This causes evaporation of the water in the tank 45 20 whereby the desired moisture content is maintained in the air adjacent the mold. The heat supplied by the steam pipes 21 causes partial curing of the molded articles. If too much heat is supplied, the concrete may exhibit undesired 50 55

expansion or "fluffing." This impairs the quality of the finished product. To prevent this result I subject the molded articles, after partial curing, to vibration or compression by any suitable means, and thus again densify and compact the articles in the mold.

When the articles have set sufficiently to be self supporting, which condition is attained in a relatively short time, because of the rapidity at 10 which curing proceeds in the temperature maintained adjacent the mold, I partially remove the articles from the chambers of the mold, by means of the apparatus described and claimed in the parent application referred to above. 15 This breaks the bond between the articles and certain of the mold parts and thereby facilitates the final removal of the articles from the mold.

A final curing chamber is located alongside 20 the mold 19 and may conveniently take the form of a liftable, open-bottomed box 23. Successive layers of articles formed in the mold 19 are deposited over a water tank 24 having steam pipes 25 therein and enclosed by the cover 23 25, forming a final curing chamber. Steam is supplied to the pipes 25 in such manner as to maintain in the chamber a temperature even higher than that to which the articles were initially subjected, e. g., 225° to 250° F. I have found 30 that molded concrete articles, after initial curing, may safely be exposed to such temperature to accelerate the completion of the curing cycle without danger of expansion or "fluffing."

On completion of the curing, the articles are 35 separated from the mold portions which were removed from the mold with them to provide a unitary liftable mass including a plurality of articles, and piled on skips 26 for further handling en masse. In order to prevent excessive 40 dehydration of the heated articles on exposure to the air, by evaporation of such free water as remains in them, I dip them in a tank 27 of cold water. This dipping operation chills the blocks and thus prevents excessive dehydration on subsequent exposure to the air. Heat-exchange 45 pipes 28 may be connected to a convenient source of heating or cooling fluid to maintain the bath in the tank 27 at the proper temperature. Instead of plain water, the tank 27 may 50 contain a coloring, sealing or hardening liquid. Since the pores of the articles are open when they are heated, such liquids will readily penetrate the articles on dipping. After dipping, the skip loads of articles are piled as indicated at 55 29 for gradual shrinkage. This process as previously carried out required a considerable length of time. I reduce the time required for shrinkage by storing the articles in the same room in which they are molded and cured and 60 close enough to the heated molding and curing chamber so that the waste heat therefrom maintains the blocks in storage at a temperature of above 40° F. and accelerates the shrinkage process.

65 The articles produced in accordance with the invention are characterized by a striking appearance. They are almost pure white, unless artificially colored, and are entirely free from the discolorations usually characterizing such articles as made heretofore. By handling the blocks en masse, I avoid the danger of breakage or chipping which exists when the blocks are handled

individually. This procedure is carried out even in delivering the articles to the job, as the loaded skips 26 may conveniently be placed on a delivery truck and the blocks removed at the job in the most convenient location. The empty skips are then returned from the job for re-loading.

The vibration of the mold after initial curing of the articles therein produces a stronger product with a lower absorption coefficient than has 10 been obtainable heretofore. This is because the vibration eliminates the cells formed in the cement paste by the quick hydration thereof resulting from heat applied in the curing. As already indicated, the chilling of the blocks when 15 cured prevents excessive loss of moisture therefrom and also permits the application of coloring, sealing or hardening agents. The sudden chilling of the articles produces no observable ill effects. By protecting the articles during aging 20 against abnormally low temperatures, the strength of the finished article is increased and an attractive color imparted thereto, viz., almost a pure white.

While I have illustrated and described herein 25 but a preferred practice of my method, it will be understood that changes in the procedure disclosed may be made without departing from the spirit of the invention or the scope of the appended claims.

I claim:

1. In a method of making concrete articles, the steps including pouring concrete into the mold, vibrating the mold, heating the mold and the concrete therein, and vibrating the mold and 35 its contents after partial setting of the latter.

2. In a method of making concrete articles, the steps including molding the articles, subjecting the articles to heat to accelerate the hydration of the cement in the concrete by the 40 available water, and, before elimination of all the free water, wetting the articles with a liquid at a temperature substantially below that to which the articles are heated, while they are hot from the curing, thereby chilling them and inhibiting excessive dehydration.

3. The method defined by claim 2 characterized by dipping the articles in the water.

4. In a method of making concrete articles, the steps including depositing concrete in a mold, 50 heating the concrete in the mold, thereby effecting a partial curing of the article, vibrating the article to reduce the voids formed by the removal of surplus water in curing, removing the article from the mold, subjecting it to further heating adjacent the mold to complete the curing, wetting the article while hot from the curing with water at a temperature below that of the article, thereby cooling it and inhibiting excessive dehydration, and storing the article near 55 enough to the mold so that the waste heat from the curing operation expedites volume change in the article in storage.

5. In a method of making concrete articles, the steps including depositing a cementitious mix in a mold, curing the formed articles by applying heat to the mold, said heat driving off surplus water in the articles, and reducing the voids left by the removal of said surplus water, by vibrating the articles.

ALBERT HENDERSON.